

April 10, 1945.

E. BASSIST

2,373,287

METHOD OF PREPARING A PRINTING PLATE

Filed July 27, 1943

*Fig. 1.*



*Fig. 2.*



*Fig. 3.*



*Inventor:*

Ellis Bassist

*By* *Wm. H. Hamill*  
*Attorney*

## UNITED STATES PATENT OFFICE

2,373,287

## METHOD OF PREPARING PRINTING PLATES

Ellis Bassist, Brookline, Mass., assignor to William Craig Toland, trustee, Brookline, Mass.

Application July 27, 1943, Serial No. 496,329

6 Claims. (Cl. 101—149.2)

This invention relates to a planographic printing plate and its method of preparation, and more especially to a "direct-image" type of plate.

By the term "direct-image printing plate" is meant a planographic printing plate in which greasy material, constituting printing portions of the plate, is directly applied to the surface of the plate, as by typewriting, hand drafting and the like, as distinguished from photolithographic plates in which printing portions are formed by photographic methods. While not being limited thereto, the invention is particularly directed to plates formed by direct application of printing portions with a typewriter to sheets of paper.

An object of the invention is to improve planographic printing plates and methods of preparation therefor, and to devise a "direct-image" type of paper printing plate which is simple, cheap and efficient, and which affords greatly improved quality of reproduction and marked increase in durability.

The nature of the invention and its objects will be more fully understood from the following description of the drawing and discussion relating thereto.

In the accompanying drawing:

Fig. 1 is an enlarged cross-sectional view illustrating a sheet material employed in forming the plate of the invention;

Fig. 2 is a fragmentary plan view illustrating a step in preparing the plate of the invention; and

Fig. 3 is a fragmentary plan view illustrating another step resulting in a finished printing plate.

In connection with forming typewritten printing portions on a printing plate base, difficulty is experienced in getting enough of the typewriter ribbon ink transferred to furnish a sufficiently strong ink body for a printing image. It is also difficult to anchor the ink body to the base so that it will not be separated or dislodged, and finally it is difficult to maintain the ink body in a sufficiently hardened condition so that it will not smudge and its original outline and character lost.

The plate of the invention is characterized by printing images or printing portions which, when formed by typewriting as well as by other modes of application, present a relatively heavy ink body, which are very tenaciously attached to the base, and finally which are of a relatively tough, durable character adapted to preserving and reproducing accurately the original subject matter.

In general, these characteristics of a relatively heavy ink body hardened to resist smudging and strongly bonded to a supporting base, are obtained

by introducing into a normally water-receptive base limited amounts of an agent for imparting a superficial grease-retentive character to the surface of the base. The grease-retentive surface is utilized to insure transfer of a relatively heavy typewritten image. The entire surface of the plate is then treated with a lithographic etching mixture which eliminates the superficial grease-retentive character from those areas surrounding the typewritten image. At the same time the lithographic etching agent cooperates with the impregnating agent in the base to convert the ink image to an exceedingly tough ink body fixed in the base.

Referring more in detail to the invention, Fig. 1 illustrates a sheet of paper 1 which preferably consists of a strong kraft paper impregnated with a sizing adapted to impart wet strength to the paper. Examples of a suitable sizing for this purpose are resinous or colloidal materials such as polyvinyl alcohol, gelatin, and the like. The paper also preferably includes water-repellent material applied at either side thereof.

The paper at its outer side further includes a lithographic printing coating 2 of polyvinyl alcohol and a filler. The polyvinyl alcohol in this case constitutes a water-receptive medium, and the filler acts as a bodying agent in the coating. Other lithographic printing coatings may be employed, as for example mixtures of albumen and other colloids with fillers, or colloidal materials alone, or other combinations.

In accordance with the invention, the water-receptive coating 2 is provided with a surface of superficial grease-receptive character obtained by treating the coating with a chemical reagent. A preferred example of chemical agent is a tannin or tannic acid. Fig. 2 diagrammatically illustrates a plate having a water-receptive coating 2, and Fig. 3 illustrates the coating 2 after treatment with tannic acid. In applying a chemical reagent to the coating 2, it is essential to carry out a limited degree of impregnation, and as illustrative of suitable concentrations for effecting a limited impregnation, the use of weak solutions, such as solutions of from 1% to 5% concentration of tannic acid, may be employed, with a 3% solution giving optimum results.

The use of a limited amount of the tannic acid is necessary in order to control the degree of grease-retentive character which is to be built up in the colloid surface. Treatment of the polyvinyl alcohol with tannic acid results in a chemical change in the nature of a hardening action as is more fully explained at a later point in the

specification. By utilizing increasing amounts of the tannic acid, grease-retentive character may progress to a point where it becomes permanently established.

While a primary object of the invention is to build up a sufficiently strong grease-retentive character so that the plate may receive and hold relatively large amounts of ink applied from a typewriter ribbon, it is nevertheless equally important to be able to eliminate the grease-retentive character in those areas which are not covered with typing, and to develop at these points a completely water-receptive grease-repellent character which will positively reject greasy ink and thus prevent "scumming." Also it is necessary to effect this change without impairing the character of the typewritten subject matter which has already been applied to the plate.

These conditions determining the amount of grease-retentive character to be provided are satisfied by utilizing a chemical reagent of the strength and type noted with a water-receptive sheet material and also by the use of a lithographic etch as disclosed in the following description of the method of forming a printing plate from the base of the invention.

A preferred method of employing the impregnated paper of the invention consists in utilizing it in sheets of sizes suitable for typing as 8½ x 11" and the like. A sheet of this character is inserted in a typewriter and typewritten subject matter applied thereto, making use of a special typewriter ribbon which is impregnated with an ink containing a fatty acid such as oleic acid.

The typed sheet is then removed and treated with a lithographic etch containing a mixture of an iron compound and chromic acid. The typewritten subject matter forms printing portions while the areas surrounding the inked subject matter accept water and form non-printing or ink-rejecting portions. The plate may thereafter be inked and printed in the usual manner.

The tannic acid impregnated in the coating 2 is especially effective in establishing a superficial grease-receptive character on the surface of the coating 2 so that the coating may accept relatively large amounts of greasy printing ink from a typewriter ribbon, and thereby form a strong printing image which can be inked and printed in a lithographic printing press. It is pointed out that the use of the tannic acid in the manner noted is generally illustrative of a method of incorporating into a water-receptive planographic base an agent which will exert a superficial hardening and produce a modified ink-receptive character.

It is known that tannic acid is an insolubilizing agent and hardening agent for colloids in general and for polyvinyl alcohol in particular, and it is understood that upon incorporating the tannic acid into the polyvinyl alcohol coating, a chemical reaction takes place with the formation of tannates of polyvinyl alcohol. As compared with polyvinyl alcohol, such tannates are less water-receptive and more grease-receptive. In those cases where small amounts of tannic acid, such as is obtained from a 3% solution, are impregnated in the coating, there is developed a limited hardening only which produces a superficial grease-receptive character.

Of further importance is the limited character of the hardening exercised by the tannic acid. The surface of the polyvinyl alcohol coating is

most affected with little hardening progressing downwardly into the coating. On account of this only a superficial grease-retentive character is developed which may be dissipated by treatment with the etching mixture of ferric chloride and chromic acid. It is believed that the lithographic etch may either toughen the polyvinyl alcohol and convert it into a water-swollen state, at which time grease-receptive character is thrown off, or the chromium compound may remove the tannates of polyvinyl alcohol chemically, while causing the underlying polyvinyl alcohol to become water-swollen. This explanation is given by way of supposition only and the invention is not intended to be limited in any way thereby. It is again pointed out that equally important with developing grease-retentive character in the base, is elimination of this grease-retentive character after an image is applied, and this important result is achieved by the use of a chemical reagent in the manner noted.

In addition to functioning as an agent for modifying grease-retentive character of paper, the tannic acid provides a further highly desirable result by cooperating with the mixture of ferric chloride and chromium compound to provide a substantial hardening of the greasy ink image. The manner in which this hardening is accomplished is not fully understood although it is suggested that there is a reaction between the fatty acid of the ink (oleic acid), the tannic acid and the iron chloride and chromic acid mixture. Whatever the explanation may be, the combined action of the tannic acid and the lithographic etch converts the ink to a tough rubbery mass which is exceedingly durable. This enables a plate made in this way to stand up under several thousand impressions as compared with a few impressions which might be obtained from printing images of typewritten subject matter prepared in the usual way.

Still another important point in connection with the use of the tannic acid in the coated paper consists in slightly varying the strength of the tannic acid solution applied to the paper coating for the purpose of modifying the shade or weight of the printing image to be reproduced. The printing image formed by typewriting can be obtained in either a light or dark copy in accordance with the strength of tannic acid present in the coating. This is an advantage in instances where it is desired to reproduce typewritten subject matter of either light or dark character.

Upon applying tannic acid to most papers and then allowing the paper to dry, the latter curls upon itself and is difficult to handle. By the use of water-repellent coatings at either side of the paper, as noted earlier in the specification, curling is eliminated and the paper is maintained in a perfectly flat state. This is an advantage during the operation of converting the paper into a printing plate and affords a convenient surface upon which to work.

A modification of the invention consists in a sheet of paper which does not include the colloid coating 2 but is provided with a water-receptive surface. One example of a paper of this nature is a parchment paper, that is, a paper which has been digested with acid. Another example of paper of this character is a fiberboard or zinc chloride treated paper. Other types of base materials or coated papers, as well as plastics and resinous sheet materials may also be employed.

In any of these modified paper or similar base

materials, the tannic acid or other impregnating agent is utilized in the same manner as described in connection with the polyvinyl alcohol and filler coating, that is, the tannic acid is impregnated directly in the treated paper or plastic as the case may be, and typewritten subject matter may then be applied in the manner described. It is further intended that the base may be utilized to form a plate by hand drafting or even photographic methods when this may be found desirable.

In place of the tannic acid, it may be desired to employ various other hardening agents for polyvinyl alcohol, as for example chromic acid or ammonium dichromate, formaldehyde, borates and others.

These hardening agents are not regarded as being as satisfactory as the tannic acid in some respects, although they are all adapted to limited use in developing grease-receptive character and may be desired to be employed in conjunction with an etch such as the ferric chloride chromic acid mixture.

For instance, chromium compounds in weak concentrations may be used to increase grease-receptive character which may be reconverted to water-receptive character with the etch. However, the chromium compounds should be used soon after impregnation as after standing for periods of several weeks or longer, it is more difficult to develop the water-receptive character.

It may also be desired to utilize the etch independently of any impregnating agent in the base material. One example of such a use consists in typing with a heavy typewriter ink upon a surface which is perfectly dry and free from moisture so that there is no tendency on the part of the paper to reject the ink. The etch here develops non-printing portions which are equally as good as those obtained by treatment of a tannic acid impregnated base. However the printing portions are not as durable or as satisfactory in other ways as those obtained by the combined use of the etch and tannic acid impregnated in the base. Some modification may also be resorted to in the lithographic etch. For example an aqueous mixture of ferric chloride alone may be used to secure desirable hardening of the greasy ink image. Similarly the chromium compound may be utilized separately of the ferric chloride, and various other combinations may be employed such as those containing other iron compounds as ferric sulphate, iron oxide, and others.

The use of tannic acid and an iron compound, such as ferric chloride, as well as a chromium compound, to form grease-retentive printing portions in a direct-image plate, may be carried out in other ways. For example in hand drafting as by a pen, a greasy ink mixture is not as readily applied since the greasy ink will not flow freely from a pen point. In this type of work, it has been found that a mixture made up of tannic acid, water, ferric chloride, chromic acid and an agent, such as hydrogen peroxide, provides a free-flowing ink, which, when dried on a surface such as paper or the coating 2, will form a hard ink-receptive basis.

The tannic acid, iron compound and chromium compound, while not of themselves being greasy, convert the base surface, as for example the coating 2, to a hardened grease-retentive state, and at the same time the several reagents, due to chemical reaction, are darkened

and upon being applied to the surface of the base, gradually turn to a dense black color.

It is pointed out that when drawing with a pen which is inked with an ink mixture such as that described, much greater amounts of ink may be transferred to the paper than are possible from the use of a typewriter ribbon, and thus a sufficiently strong image may be produced. The writing mixture of tannic acid, iron chloride and chromic acid is not, of course, as suitable as a greasy ink for use in impregnating a typewriter ribbon and in making typewritten images.

A further modification of ink which may be employed consists in an emulsified product containing both a fatty acid and aqueous materials thoroughly mixed together. The emulsion, which may or may not include any of the chemical reagents referred to, is adapted to adhere more readily to water-receptive surfaces by reason of the presence of small amounts of aqueous materials in the emulsion. The result of this is to improve transfer of printing ink from a typewriter ribbon to water-receptive surfaces.

It should be observed that the method of the invention provides for the development of a superficial grease-retentive character in a water-receptive base which facilitates application of an ink image thereto, and at the same time the method of the invention provides for removing or dissipating the superficial grease-retentive character after application of the printing image, and at a time when the printing image itself may be converted to a hard durable mass while water-receptive character is being revived in the non-printing portions of the plate. The printing plate resulting from this method is formed with printing portions and non-printing portions in accordance with the usual lithographic principle of printing. The printing portions include tannates of polyvinyl alcohol (in the case of a polyvinyl alcohol coated plate) and a chemically hardened greasy ink. The non-printing portions of the plate consist of polyvinyl alcohol which has been toughened at its surface by chemical treatment but which nevertheless exhibits a water-swollen condition which provides a completely water-receptive character and which positively rejects ink with no occurrence of scumming.

In forming a lithographic printing image, the typewriter action and typewriter ribbon will apply only a very small amount of typewriter ink to the surface of the paper, and the paper itself must be of a type which takes ink easily, is readily inserted in the machine, and otherwise dealt with. In view of this, formation of printing plates from typewritten subject matter has been unsatisfactory, and at best, plates of questionable quality and very limited life have been produced.

The impregnated sheet material of the invention substantially aids in overcoming these difficulties, by temporarily increasing the grease-receptive character of the paper and by thus insuring that a satisfactory amount of ink may be applied. The impregnating agent in the paper also cooperates with other chemical etching agents referred to in hardening the ink and providing for many impressions being made, as for example 25,000 impressions and more. In addition, the paper is very easy to use and is not subject to difficulties in connection with development of the printing image so that an unskilled operator may very quickly prepare the

printing image for use in a printing press. Various other advantages are also present in connection with the paper sheet material of the invention such as light weight, low cost, and the like.

While I have shown a preferred embodiment of my invention, it should be understood that various changes and modifications may be resorted to, in keeping with the spirit of the invention as defined by the appended claims.

I claim:

1. That improved process which comprises applying to a sheet material having a water-receptive surface a solution of tannic acid, applying an ink image on the surface, said ink containing oleic acid, treating the image with a lithographic etching mixture which contains ferric chloride.

2. The improved process which comprises applying to a sheet material having a water-receptive surface a solution of tannic acid, applying an ink image on the surface, said ink containing oleic acid, and treating the image with a lithographic etching mixture which contains ferric chloride, chromic acid and gum arabic.

3. That improved process which comprises applying to a sheet material having a water-receptive surface a solution of tannic acid, applying an ink image on the surface, said ink containing oleic acid, and treating the image with

a lithographic etching mixture which contains an iron compound, a chromium compound and an aqueous material.

4. That improved process which comprises providing a sheet of paper with a coating of water-swellable polyvinyl alcohol and a filler, impregnating the coating with tannic acid, transferring typewritten subject matter to the coating with a typewriter ribbon which contains a fatty acid ink, and then etching the plate with a mixture of water, gum arabic, perchloride of iron and a chromium compound.

5. That improved process which comprises providing a sheet material, impregnating the sheet material with a chemical agent, applying an ink image on the impregnated surface, treating the image with a lithographic etch which contains a chemical reagent adapted to cooperate with the said first chemical agent in hardening the image.

6. That improved process which comprises providing a sheet material, impregnating the sheet material with a chemical agent to modify its grease-receptive character, applying an ink image thereto, treating the entire surface of the sheet material with an etch which cooperates with the said first agent to harden the image.

ELLIS BASSIST.